# EUROPEAN PATENT SPECIFICATION

(11) **EP 3 189 187 B1**
(45) Date of publication and mention of the grant of the patent: **09.06.2021**
(21) Application number: 15775804.6
(22) Date of filing: 31.08.2015
(51) Int. Cl.: D06M 10/10, D06M 15/03, D06M 13/188, D06M 13/192

(54) **SIZING COMPOSITION FOR FIBERS, YARNS AND/OR FABRICS AND PROCESS FOR PREPARING SUCH SIZING COMPOSITION**
SCHLICHTEZUSAMMENSETZUNG FÜR FASERN, FÄDEN UND/ODER GEWEBE UND VERFAHREN ZUR HERSTELLUNG SOLCH EINER SCHLICHTEZUSAMMENSETZUNG
COMPOSITION D'ENCOLLAGE POUR FIBRES, FILS ET/OU TISSUS, ET PROCÉDÉ DE PRÉPARATION DE CELLE-CI

(30) Priority: 03.09.2014 IT MI20141534; 23.02.2015 IT MI20150270
(43) Date of publication of application: 12.07.2017
(73) Proprietor: Canepa S.p.A., 22020 San Fermo della Battaglia (CO) (IT)
(72) Inventor: CANEPA, Elisabetta, I-22020 San Fermo della Battaglia (CO) (IT)
(74) Representative: Simino, Massimo
(86) International application number: PCT/IB2015/056588
(87) International publication number: WO 2016/034997

(56) References cited:
- EP-A1- 1 897 893
- EP-A1- 2 105 459
- WO-A1-2007/083870
- WO-A1-2013/057723
- WO-A1-2015/159262
- IT-A1- MI20 121 778

## Description

The present invention relates to a sizing composition for fibers and yarns and/or fabrics made from such fibers, particularly for natural animal fibers, vegetable fibers, synthetic polymer fibers, man-made natural polymer fibers, continuous filaments of animal origin and/or discontinuous filaments of animal origin, to be used at a pure state or blended together.

As used herein, the term weaving is generally used both for designating warp-and-weft weaving and knit-weaving.

As used herein, for example:
- thin yarns are intended to cover yarns having a yarn count ranging from 40 to 200 Nm, more preferably a yarn count of 65 Nm or more;
- animal fibers are intended to cover fleece or hair fibers (such as wool, alpaca, vicuna, cashmere, etc.);
- continuous filaments of animal origin are intended to cover filaments obtained by reeling from whole cocoons (such as silk);
- discontinuous filaments of animal origin are intended to cover filaments obtained by unravelling from defective cocoons (such as waste silk);
- vegetable fibers are intended to cover all the fibers obtained from plants, shrubs, inflorescences, roots, leaves (such as cotton, flax, hemp, jute, coir, ramie, bamboo, and others);
- synthetic polymer fibers are intended to cover, for example, polyamide, polyester, acrylic, polypropylene fibers, and others;
- man-made natural fibers are intended to cover, for example, rayon viscose, modal, acetate, cupro, lyocell, and others.

The technique of applying a sizing composition to yarn fibers has been long known and is generally used to improve weavability of yarns, particularly thin yarns which are inherently difficult to weave as weft and/or warp yarns due o their thinness and their low tensile breaking load.

Sizing compositions can be generally removed from fabrics by suitable hydrolysis processes (e.g. acid, oxidizing or enzymatic hydrolysis) or are watersoluble such that they may be entirely removed from the fibers by appropriate finishing processing steps, such as washing or dyeing.

It shall be noted that additional needs are felt, such as:
- enhancing the mechanical properties of abrasion resistance of thin yarns, while reducing mechanical friction between weft yarns and warp yarns, for trouble-free weaving;
- developing an environment-friendly and low-power-consumption process for making a yarn having improved weavability features;
- developing a process for making a yarn having improved features in terms of resistance to pilling, felting and rubbing, as well as superior mechanical properties while maintaining the desired softness, volume, brightness and lightness features;
- developing a process for making a yarn having improved dye affinity, or improved affinity for the later finishing steps, such as printing.

In view of the above needs, sizing compositions have been tested, which could have a lasting effect on the fibers upon which they are applied, i.e. remain on the fibers even after the above mentioned finishing steps or after successive repeated washing steps. A substantially permanent presence of the sizing composition on the fibers of a yarn or a knit will allow fulfillment of the above mentioned additional needs.

For example, the use of sizing compositions comprising chitosan has been suggested, wherein, after application to the fibers, the chitosan contained in the sizing composition is crosslinked, whereby such chitosan generates a crosslinked polymer which remains permanently anchored to the fibers.

Chitosan is a natural polymer derived from chitin, which is a polysaccharide contained in the exoskeleton of crustaceans, and is a nature-renewable material, since it is obtained from food industry by-products.

It shall be noted that the chitosan-based reinforcement product used in the sizing composition has much better sizing properties than other natural substances.

The above chitosan crosslinking step has the purpose of imparting a considerable physical-mechanical resistance to the fibers upon which chitosan is applied, while ensuring a long-lasting sanitization effect, resisting many repeated washes with hot and/or soapy water, as well as a considerable improvement in the dye affinity, of the treated fibers.

Conversely, the presence of the crosslinked chitosan and/or derivatives thereof on the fibers is likely to impart an excessive stiff feel to the fibers of the fabric or knit, and the fabric or knit are no longer soft and supple, i.e. are said to have a "hard feel", even when it is formed with thin fibers, e.g. cashmere fibers having a yarn count of 70 Nm.

Therefore, the invention is based on the problem of conceiving and providing a sizing composition that fulfills all the above mentioned needs, without imparting stiffness to the fibers of the fabric or knit upon substantially permanent application of such sizing composition to the fibers due to crosslinking of chitosan and/or derivatives thereof, contained in the sizing composition.

This problem is solved by a sizing composition as defined in claim 1.

In a further aspect, another problem consists in conceiving a method of preparing a sizing composition comprising chitosan, which is effective and economic and can be easily implemented in a manufacturing process without requiring excessively long processing/preparation times, while providing a sizing composition in which chitosan is finely dissolved.

According to the invention, this additional technical problem is solved by means of a process as defined in claim 8 for preparing a sizing composition of the invention.

In a further aspect, the invention also relates to a process as defined in claim 14 for crosslinking chitosan and/or derivatives thereof contained in the sizing composition of the invention on fibers impregnated with such sizing composition.

According to the invention, the sizing composition to be used for sizing the fibers (particularly natural animal fibers, vegetable fibers, synthetic polymer fibers, man-made natural polymer fibers, continuous filaments of animal origin and/or discontinuous filaments of animal origin, to be used at a pure state or blended together) or the yarns, fabrics or knits obtained from such fibers is a sizing composition comprising chitosan and/or derivatives thereof.

Advantageously, the chitosan and/or derivatives thereof as used for preparing the sizing composition of the invention have:
- a molecular weight ranging from 120,000 Da to 180,000 Da, preferably a molecular weight of the order of 150,000 Da, such molecular weight being expressed as viscosity average molecular mass, or Mv
- a degree of deacetylation of 70-90%, preferably a degree of deacetylation of 75-85% and/or
- a viscosity at ambient temperature (indicatively a temperature of about 25°C, Brookfield viscosity) of 20-200 cps, 1% w/w chitosan in 1% w/v acetic or citric acid.

The chitosan and/or derivatives thereof are dissolved in a 3% to 9% w/v organic acid solution, with a pH of less than 6.5.

Preferably, the chitosan and/or derivatives thereof are dissolved in a 3% to 9% w/v acetic acid or citric acid solution, 3-9% v/v.

By way of example only, pyruvic acid and tartaric acid may be used as further organic acids. Preferably, the chitosan and/or derivatives thereof in the sizing composition are in a solid state (e.g. powder, granules or flakes) or in a fluid state (e.g. in the form of a high-density paste), before being dissolved by agitation and/or by dispersion in said sizing composition.

Preferably, the above mentioned sizing composition also comprises starch and/or fish glue at a ratio of 1:1 to the amount of chitosan and/or derivatives thereof.

To facilitate UV crosslinking of chitosan and/or derivative, the above mentioned sizing composition is enriched with additional double-bond monomers crosslinking agents comprising acrylic monomers with low environmental impact, added in an amount substantially equal to the w/v percent of chitosan and/or derivatives thereof in the sizing composition.

Preferably, the above mentioned polycarboxylic acids comprise citric acid added in an amount not more than 2% w/v based on the amount of dry chitosan in the sizing composition.

Furthermore, crosslinking of chitosan and/or derivatives thereof, applied to the fibers, may be obtained by chemical and/or thermal treatment, with the sizing composition bath including formulations containing double-bond acrylic monomers, e.g. 2-hydroxy ethyl methacrylate (HEMA), and optionally polycarboxylic acids, such as citric acid.

Advantageously, before being used for sizing fibers, the above mentioned sizing composition undergoes a dissolution step, by agitating the chitosan and/or derivatives thereof in the sizing composition for a period of more than 10 hours, and preferably the sizing composition undergoes agitation for a period of 12 hours to 24 hours, at a temperature ranging from 60°C to 80°C, preferably a temperature of about 70°C.

In a different and more advantageous production mode, alternative to the above described dissolution by agitation, the above mentioned sizing composition is prepared by submitting the sizing composition to be prepared to a step of dissolution by dispersion, during which the chitosan that has been added into the sizing composition is dissolved after being finely dispersed in the sizing composition.

The above mentioned step of dissolution by dispersion of the chitosan and/or derivatives thereof is carried out by dispersion means that are adapted to achieve fine dispersion of the chitosan and/or derivatives thereof in the bath (i.e. the sizing composition) by high-speed impacts with the solid chitosan particles contained in the bath.

These dispersion means comprise at least one COWLES-type impeller or an impeller having blades, particularly, but without limitation, a toothed-disk impeller, with the teeth formed of blades, preferably having a sawtooth shape. According to preferred embodiment, these blades or teeth are placed at the outer peripheral edge of the impeller disk and/or project out of both sides of said disk.

According to a preferred embodiment, the COWLES-type impeller or the impeller with blades comprises a varying number of peripheral teeth, e.g. ranging from ten to forty. The number of teeth of the impeller varies, namely increases, with the outside diameter of the impeller.

The outside diameter of the COWLES-type impeller or the impeller with blades is at least 5 cm, and may be up to 100 cm in the case of large dispersers. Preferably, the diameter of the COWLES-type impeller or the impeller with blades ranges from 12 cm to 40 cm.

In short, the bath in which the chitosan and/or derivatives thereof are added in a solid state (e.g. powder, granules or flakes) or in a fluid state (e.g. in the form of a high-density paste) is contained in a tank of a disperser in which said COWLES impeller or said impeller with blades is rotatably actuated at high speed, i.e. at a peripheral speed of rotation of the impeller of 10 meters/second or more and less than 40 m/second, preferably at a peripheral speed of the impeller of 13-32 meters/second. This will afford a surprising and effective dispersion of the particles of chitosan and/or derivatives thereof in the bath, to complete and rapid dissolution of the particles of chitosan and/or derivatives thereof in the bath, leading to the formation of the sizing composition of the invention.

According to a preferred embodiment, the inside diameter of the above mentioned tank is twice to six times the maximum outside diameter of the COWLES-type impeller or the impeller with blades. More preferably, the inside diameter of the above mentioned tank is three to four times the maximum outside diameter of the COWLES-type impeller or the impeller with blades, which will provide an advantageous condition when the inside diameter of the tank is about three times the maximum outside diameter of the COWLES-type impeller or the impeller with blades.

Advantageously, complete dispersion of particles of chitosan and/or derivatives thereof in the bath, which is achieved using a COWLES impeller or an impeller with blades, and leads to the dissolution of such particles of chitosan and/or derivatives thereof in the bath, and to the formation of the sizing composition comprising chitosan and/or derivatives thereof, is obtained in very short process times, indicatively also less than one hour, e.g. of the order of 35-45 minutes, with no need to extend said dispersion step to multiple hours, as required by the dissolution by agitation as described above.

It shall be further noted that the above mentioned complete dissolution by dispersion of particles of chitosan and/or derivatives thereof in the bath, which is achieved using a COWLES impeller or an impeller with blades, can be also achieved at ambient temperature, indicatively also at temperatures of about 15°C, optimal results being also achievable with temperatures of less than 40°C. Therefore, said dissolution by dispersion of chitosan and/or derivatives thereof in the bath does not require extended heating at temperatures of the order of 60-80°C, as required in dissolution by agitation as described above.

Advantageously, the crosslinking of chitosan and/or derivatives thereof contained in the above mentioned sizing composition on fibers impregnated with such sizing composition is obtained by exposing the fibers impregnated with said sizing composition to the radiation of a UV lamp.

Preferably, the step of crosslinking on the fibers impregnated with chitosan and/or derivatives thereof contained in such sizing composition is obtained by exposing the fibers impregnated with said sizing composition to the radiation of a UV lamp:
- having a power of 400W to 600W, preferably a power of about 500W, and
- having an intensity of 10 mV/cm² to 30 mV/cm², preferably an intensity of about 20 mV/cm²,
for an exposure time ranging from 20 to 80 seconds, preferably for an exposure time ranging from 30 to 65 seconds, at a distance from the UV lamp ranging from 15 cm to 30 cm, preferably at a distance of the order of 20 cm from the UV lamp.

Preferably, the above mentioned step of exposure of the impregnated fibers to the radiation of the UV lamp is preceded by a step of wringing, partially drying or completely drying the fibers.

Alternatively, as described above, the crosslinking of the fibers of chitosan and/or derivatives thereof, contained in the above mentioned sizing composition may be obtained by chemical treatment, possibly after a step of wringing, partially drying or completely drying the fibers.

Experimental tests proved that the use of the sizing composition of the invention for sizing the fibers, and the later step of crosslinking and/or derivatives thereof contained in the sizing composition can provide fibers, e.g. in the forms of a yarn, a fabric or a knit, that can fulfill the above mentioned needs. This is because said fibers have an amount of crosslinked chitosan and/or chitosan derivatives substantially permanently applied thereto, such amount allowing to achieve the desired beneficial effects, without causing the fibers to have a stiff or poorly soft feel.

Namely, according to the specific compounds that form the sizing composition in use, the specific method of producing such sizing composition and the specific crosslinking method, the sized fibers only have crosslinked, i.e. permanently applied, thereto, the amount of crosslinked chitosan and/or crosslinked chitosan derivatives that is required to achieve the desired effects, and the rest of the sizing composition may be removed, by desizing, with a simple washing step with water at 35-40°C or a later finishing step. Particularly, such later water washing or finishing step only removes the chitosan and/or derivatives thereof that have been crosslinked but do not adhere to the fibers.

In the light of the above disclosure, the sizing composition as described above, and the process of preparing the sizing compositionof the invention and the crosslinking process in use, can fulfill the above mentioned needs, while obviating the lamented drawbacks.

The above disclosure is susceptible to a number of changes and variants within the inventive concept, as outlined by the annexed claims.

## Claims

1. **A sizing composition** for fibers and yarns and/or fabrics made from such fibers, particularly for natural animal fibers, vegetable fibers, synthetic polymer fibers, man-made natural polymer fibers, continuous filaments of animal origin and/or discontinuous filaments of animal origin, to be used at a pure state or blended together, wherein said sizing composition comprises chitosan and/or derivatives thereof, wherein:
- said chitosan and/or derivatives thereof have a molecular weight Mᵥ ranging from 120,000 Da to 180,000 Da, preferably a molecular weight Mᵥ of the order of 150,000 Da, with a degree of deacetylation of 70-90%, and an ambient temperature viscosity of 20-200 cps with 1% w/w chitosan in 1% w/v acetic or citric acid,
**characterized in that:**
- said sizing composition comprises an organic acid solution with a pH of less than 6.5 at 3-9% v/v, in which 3% to 9% w/v of said chitosan and/or derivatives thereof are dissolved:
• by agitation or
• by a dispersion step that is carried out using a COWLES-type impeller or an impeller with blades, preferably a sawblade impeller, which can impact the solid particles of chitosan and/or derivatives thereof at high speed, and
- to facilitate UV crosslinking of chitosan and/or derivative, said sizing composition is enriched with additional double-bond monomers crosslinking agents comprising acrylic monomers with low environmental impact added in an amount equal to the w/v percent of chitosan and/or derivatives thereof in the sizing composition.

2. A sizing composition as claimed in claim 1, wherein to facilitate UV crosslinking of chitosan and/or derivative, said sizing composition is enriched with additional crosslinking agents comprising:
• drying oils, preferably linseed oil consisting of oleic and linoleic acid, and/or
• polycarboxylic acids.

3. A sizing composition as claimed in claim 1 or 2, wherein said organic acid solution with a pH of less than 6.5 at 3-9% v/v, is an acetic acid, a citric acid, a pyruvic acid or a tartaric acid solution.

4. A sizing composition as claimed in claim 1, 2 or 3, wherein the degree of deacetylation of said chitosan and/or derivatives thereof is 75-85%.

5. A sizing composition as claimed in claim 1, 2, 3 or 4, wherein the chitosan and/or derivatives thereof are in a solid state, preferably powder, granules or flakes, or in a fluid state, e.g. in the form of a high-density paste, before being dissolved by agitation and/or dispersion in said solution containing an organic acid with a pH of less than 6.5 at 3-9% v/v.

6. A sizing composition as claimed in any of claims 1 to 5, wherein said solution of chitosan and/or derivatives thereof in an organic acid, with a pH of less than 6.5, comprises starch and/or fish glue at a ratio of 1:1 to the amount of chitosan and/or derivatives thereof.

7. A sizing composition as claimed in any of claims 1 to 6 wherein;
- said sizing composition comprises:
- drying oils, preferably linseed oil consisting of oleic and linoleic acid, and/or
- polycarboxylic acids, preferably comprising citric acid added in an amount not more than 2% based on the amount of dry chitosan in the sizing composition.

8. **A process of preparing a sizing composition** for fibers and yarns and/or fabrics made from such fibers, particularly for natural animal fibers, vegetable fibers, synthetic polymer fibers, man-made natural polymer fibers, continuous filaments of animal origin and/or discontinuous filaments of animal origin, to be used at a pure state or blended together, wherein said sizing composition comprises:
- chitosan and/or derivatives thereof having a molecular weight Mv ranging from 120,000 Da to 180,000 Da, preferably a molecular weight Mv of the order of 150,000 Da, with a degree of deacetylation of 70-90%, and an ambient temperature viscosity of 20-200 cps with 1% w/w chitosan in 1% w/v acetic or citric acid and
- an organic acid solution with a pH of less than 6.5 at 3-9% v/v, in which 3% to 9% w/v of said chitosan and/or derivatives thereof are dissolved, wherein said sizing composition undergoes a step of dissolution by dispersion carried out by dispersion means that are adapted to achieve fine dispersion of the chitosan and/or derivatives thereof contained in the sizing composition by high-speed impacts with the solid particles of chitosan and/or derivatives thereof contained in the bath, to dissolution of said solid particles of chitosan and/or derivatives thereof in the bath, said dispersion means for carrying out said step of dispersion of chitosan and/or derivatives thereof comprise at least one COWLES-type impeller or a toothed-disk impeller having blades, with the teeth formed of blades, preferably having a sawtooth shape,
wherein to facilitate UV crosslinking of chitosan and/or derivative said sizing composition is enriched with additional double-bond monomers crosslinking agents comprising acrylic monomers added in an amount equal to the percent of chitosan and/or derivatives thereof in the sizing composition.

9. A process of preparing a sizing composition as claimed in claim 8, wherein said step of dispersion of chitosan and/or derivatives thereof is carried out by introducing the bath in which chitosan and/or derivatives thereof have been added in a solid or fluid state, into a tank of a disperser in which said COWLES impeller or said impeller with blades is rotatably, preferably at a peripheral speed of rotation of the impeller of more than 10 meters/second and less than 40 m/second, preferably at a peripheral speed of the impeller of 13-32 meters/second.

10. A process of preparing a sizing composition as claimed in any of claims 8 to 9, wherein said chitosan and/or derivatives thereof are dissolved by agitation or by dispersion in said sizing composition from a solid state, preferably powder, granules or flakes, or from a fluid state, preferably in the form of a high-density paste.

11. A process of preparing a sizing composition as claimed in any of claims 8 to 10, wherein said solution of chitosan and/or derivatives thereof in an organic acid, with a pH of less than 6.5 comprises starch and/or fish glue at a ratio of 1:1 to the amount of chitosan and/or derivatives thereof.

12. A process of preparing a sizing composition as claimed in any of claims 8 to 11 wherein to facilitate UV crosslinking of chitosan and/or derivative said sizing composition is enriched with additional crosslinking agents comprising:
- drying oils, preferably linseed oil consisting of oleic and linoleic acid, and/or
- polycarboxylic acids.

13. A process of preparing a sizing composition as claimed in claim 8 or 12, wherein said polycarboxylic acids comprise citric acid added in an amount not more than 2% based on the amount of dry chitosan in the sizing composition.

14. **A process of crosslinking chitosan and/or derivatives thereof** contained in the sizing composition as claimed in any of claims 1 to 7, on fibers impregnated with said sizing composition, wherein said crosslinking step is carried out by:
- by exposing the fibers impregnated with said sizing composition to the radiation of a UV lamp and
- by chemical treatment.

15. A process of crosslinking chitosan and/or derivatives thereof as claimed in claim 14, wherein said crosslinking step is carried out by exposing said fibers impregnated with said sizing composition to the radiation of a UV lamp:
- having a power of 400W to 600W, preferably a power of about 500W, and
- having an intensity of 10 mV/cm² to 30 mV/cm², preferably an intensity of about 20 mV/cm²,
for an exposure time ranging from 20 to 80 seconds, preferably for an exposure time ranging from 30 to 65 seconds, at a distance from the UV lamp ranging from 15 cm to 30 cm, preferably at a distance from the UV lamp of the order of 20 cm.

## Patentansprüche

1. **Schlichtezusammensetzung** für Fasern und Garne und/oder Gewebe, die aus solchen Fasern bestehen, insbesondere für natürliche tierische Fasern, pflanzliche Fasern, synthetische Polymerfasern, künstliche Fasern aus natürlichen Polymeren, Endlosfasern tierischen Ursprungs und/oder Nicht-Endlosfasern tierischen Ursprungs, zur Verwendung in reinem Zustand oder miteinander gemischt, wobei die Schlichtezusammensetzung Chitosan und/oder Derivate davon umfasst, wobei:
- das Chitosan und/oder die Derivate davon ein Molekulargewicht Mᵥ im Bereich von 120.000 Da bis 180.000 Da aufweisen, vorzugsweise ein Molekulargewicht Mᵥ in der Größenordnung von 150.000 Da, mit einem Deacetylierungsgrad von 70-90 % und einer Viskosität bei Umgebungstemperatur von 20-200 cps mit 1 % w/w Chitosan in 1 % w/v Essig- oder Zitronensäure,
**dadurch gekennzeichnet, dass:**
- die Schlichtezusammensetzung eine Lösung einer organischen Säure mit einem pH-Wert von weniger als 6,5 bei 3-9 % v/v umfasst, in der 3 % bis 9 % w/v des Chitosans und/oder Derivate davon folgendermaßen gelöst werden:
• durch Rühren oder
• durch einen Dispersionsschritt, der unter Verwendung eines Flügelrades vom COWLES-Typ oder eines Flügelrades mit Schaufeln, vorzugsweise eines Sägeblatt-Flügelrades, durchgeführt wird, der auf die festen Teilchen von Chitosan und/oder Derivaten davon mit hoher Geschwindigkeit auftreffen kann, und
- zur Erleichterung der UV-Vernetzung von Chitosan und/oder Derivaten davon die Schlichtezusammensetzung mit zusätzlichen Vernetzungsmitteln doppelbindiger Monomeren angereichert ist, die Acrylmonomere mit geringer Umweltbelastung umfassen, die in einer Menge hinzugefügt werden, die dem w/v-Anteil von Chitosan und/oder Derivaten davon in der Schlichtezusammensetzung entspricht.

2. Schlichtezusammensetzung gemäß Anspruch 1, wobei zur Erleichterung der UV-Vernetzung von Chitosan und/oder Derivaten die Schlichtezusammensetzung mit zusätzlichen Vernetzungsmitteln angereichert ist, die Folgendes umfassen:
• trocknungsöle, vorzugsweise Leinöl, bestehend aus Öl- und Linolsäure, und/oder
• polycarbonsäuren.

3. Schlichtezusammensetzung gemäß Anspruch 1 oder 2, wobei die Lösung einer organischen Säure mit einem pH-Wert von weniger als 6,5 bei 3-9 % v/v eine Essigsäure-, eine Zitronensäure-, eine Brenztraubensäure- oder eine Weinsäurelösung ist.

4. Schlichtezusammensetzung gemäß Anspruch 1, 2 oder 3, wobei der Grad der Deacetylierung des Chitosans und/oder der Derivate davon 75-85 % beträgt.

5. Schlichtezusammensetzung gemäß Anspruch 1, 2, 3 oder 4, wobei das Chitosan und/oder die Derivate davon in festem Zustand, vorzugsweise als Pulver, Granulat oder Schuppen, oder in flüssigem Zustand, z.B. in Form einer hochdichten Paste, vorliegen, bevor sie durch Rühren und/oder Dispergieren in der eine organische Säure enthaltenden Lösung mit einem pH-Wert von weniger als 6,5 bei 3-9 % v/v gelöst werden.

6. Schlichtezusammensetzung gemäß einem der Ansprüche 1 bis 5, wobei die Lösung von Chitosan und/oder Derivaten davon in einer organischen Säure mit einem pH-Wert von weniger als 6,5 Stärke und/oder Fischleim in einem Verhältnis von 1:1 zu der Menge an Chitosan und/oder Derivaten davon umfasst.

7. Schlichtezusammensetzung gemäß einem der Ansprüche 1 bis 6, wobei;
- die Schlichtezusammensetzung Folgendes umfasst:
- trocknungsöle, vorzugsweise Leinöl, bestehend aus Öl- und Linolsäure, und/oder
- polycarbonsäuren, die vorzugsweise Zitronensäure umfassen, die in einer Menge von nicht mehr als 2 %, bezogen auf die Menge an trockenem Chitosan in der Schlichtezusammensetzung, hinzugefügt wird.

8. **Verfahren zum Herstellen einer Schlichtezusammensetzung** für Fasern und Fäden und/oder Gewebe, die aus solchen Fasern bestehen, insbesondere für natürliche tierische Fasern, pflanzliche Fasern, synthetische Polymerfasern, künstliche Fasern aus natürlichen Polymeren, Endlosfasern tierischen Ursprungs und/oder Nicht-Endlosfasern tierischen Ursprungs, zur Verwendung in reinem Zustand oder miteinander gemischt, wobei die Schlichtezusammensetzung Folgendes umfasst:
- Chitosan und/oder Derivate davon, die ein Molekulargewicht Mᵥ im Bereich von 120.000 Da bis 180.000 Da aufweisen, vorzugsweise ein Molekulargewicht Mᵥ in der Größenordnung von 150.000 Da, mit einem Deacetylierungsgrad von 70-90 % und einer Viskosität bei Umgebungstemperatur von 20-200 cps mit 1 % w/w Chitosan in 1 % w/v Essig- oder Zitronensäure und
- eine Lösung einer organischen Säure mit einem pH-Wert von weniger als 6,5 bei 3-9 % v/v, in der 3 % bis 9 % w/v des Chitosans und/oder Derivate davon gelöst werden, wobei die Schlichtezusammensetzung einem Schritt der Auflösung durch Dispersion unterzogen wird, der durch Dispersionsmittel durchgeführt wird, die geeignet sind, eine Feindispersion des Chitosans und/oder der Derivate davon, die in der Schlichtezusammensetzung enthalten sind, durch Auftreffen mit hoher Geschwindigkeit auf die festen Teilchen des Chitosans und/oder der Derivate davon, die in dem Bad enthalten sind, zu erreichen, um die festen Teilchen von Chitosan und/oder Derivaten davon in dem Bad aufzulösen, wobei die Dispersionsmittel zur Durchführung des Schritts der Dispersion von Chitosan und/oder Derivaten davon mindestens ein Flügelrad vom COWLES-Typ oder ein Zahnscheiben-Flügelrad mit Schaufeln umfassen, wobei die Zähne aus Schaufeln gebildet sind, die vorzugsweise eine Sägezahnform aufweisen,
wobei zur Erleichterung der UV-Vernetzung von Chitosan und/oder Derivaten die Schlichtezusammensetzung mit zusätzlichen Vernetzungsmitteln doppelbindiger Monomeren angereichert ist, die Acrylmonomere umfassen, die in einer Menge hinzugefügt werden, die dem Anteil von Chitosan und/oder Derivaten davon in der Schlichtezusammensetzung entspricht.

9. Verfahren zum Herstellen einer Schlichtezusammensetzung gemäß Anspruch 8, wobei der Schritt der Dispersion von Chitosan und/oder Derivaten davon durch Einführen des Bades, in das Chitosan und/oder Derivate davon in festem oder flüssigem Zustand hinzugefügt wurden, in einen Tank eines Dispergierers durchgeführt wird, in dem das COWLES-Flügelrad oder das Flügelrad mit Schaufeln drehbar ist, vorzugsweise mit einer Umfangsgeschwindigkeit der Drehung des Flügelrades von mehr als 10 Meter/Sekunde und weniger als 40 m/Sekunde, vorzugsweise mit einer Umfangsgeschwindigkeit des Flügelrades von 13-32 Meter/Sekunde.

10. Verfahren zum Herstellen einer Schlichtezusammensetzung gemäß einem der Ansprüche 8 bis 9, wobei das Chitosan und/oder die Derivate davon durch Rühren oder durch Dispersion in der Schlichtezusammensetzung aus einem festen Zustand, vorzugsweise Pulver, Granulat oder Schuppen, oder aus einem flüssigen Zustand, vorzugsweise in Form einer hochdichten Paste, gelöst werden.

11. Verfahren zum Herstellen einer Schlichtezusammensetzung gemäß einem der Ansprüche 8 bis 10, wobei die Lösung von Chitosan und/oder Derivaten davon in einer organischen Säure mit einem pH-Wert von weniger als 6,5 Stärke und/oder Fischleim in einem Verhältnis von 1:1 zu der Menge an Chitosan und/oder Derivaten davon umfasst.

12. Verfahren zum Herstellen einer Schlichtezusammensetzung gemäß einem der Ansprüche 8 bis 11, wobei zur Erleichterung der UV-Vernetzung von Chitosan und/oder Derivaten die Schlichtezusammensetzung mit zusätzlichen Vernetzungsmitteln angereichert ist, die Folgendes umfassen:
- trocknungsöle, vorzugsweise Leinöl, bestehend aus Öl- und Linolsäure, und/oder
- polycarbonsäuren.

13. Verfahren zum Herstellen einer Schlichtezusammensetzung gemäß Anspruch 8 oder 12, wobei die Polycarbonsäuren Zitronensäure umfassen, die in einer Menge von nicht mehr als 2 %, bezogen auf die Menge an trockenem Chitosan in der Schlichtezusammensetzung, hinzugefügt wird.

14. **Verfahren zum Vernetzen von Chitosan und/oder Derivaten davon,** die in der Schlichtezusammensetzung gemäß einem der Ansprüche 1 bis 7 enthalten sind, auf Fasern, die mit der Schlichtezusammensetzung imprägniert sind, wobei der Vernetzungsschritt folgendermaßen durchgeführt wird:
- durch Belichten der mit der Schlichtezusammensetzung imprägnierten Fasern mit der Strahlung einer UV-Lampe und
- durch chemische Behandlung.

15. Verfahren zum Vernetzen von Chitosan und/oder Derivaten davon gemäß Anspruch 14, wobei der Vernetzungsschritt durchgeführt wird, indem die mit der Schlichtezusammensetzung imprägnierten Fasern mit der Strahlung einer UV-Lampe belichtet werden:
- die eine Leistung von 400 W bis 600 W, vorzugsweise eine Leistung von etwa 500 W aufweist und
- die eine Intensität von 10 mV/cm² bis 30 mV/cm², vorzugsweise eine Intensität von etwa 20 mV/cm² aufweist,
für eine Belichtungszeit im Bereich von 20 bis 80 Sekunden, vorzugsweise für eine Belichtungszeit im Bereich von 30 bis 65 Sekunden, in einem Abstand von der UV-Lampe im Bereich von 15 cm bis 30 cm, vorzugsweise in einem Abstand von der UV-Lampe in der Größenordnung von 20 cm.

## Revendications

1. **Composition d'encollage** pour des fibres et fils et/ou des étoffes fabriquées à partir de telles fibres, en particulier pour des fibres naturelles animales, des fibres végétales, des fibres polymères synthétiques, des fibres polymères naturelles de fabrication humaine, des filaments continus d'origine animale et/ou des filaments discontinus d'origine animale, destinés à être utilisés dans un état pur ou mélangés les uns avec les autres, ladite composition d'encollage comprenant du chitosane et/ou des dérivés de celui-ci, où :
- ledit chitosane et/ou lesdits dérivés de celui-ci présentent une masse moléculaire Mᵥ allant de 120.000 Da à 180.000 Da, de préférence une masse moléculaire Mᵥ de l'ordre de 150.000 Da, avec un degré de désacétylation de 70 à 90 %, et une viscosité à température ambiante de 20 à 200 cps avec 1 % m/m de chitosane dans 1 % m/v d'acide acétique ou citrique,
**caractérisée en ce que** :
- ladite composition d'encollage comprend une solution d'acide organique avec un pH inférieur à 6,5 à 3-9 % v/v, dans laquelle sont dissous 3 % à 9 % m/v dudit chitosane et/ou desdits dérivés de celui-ci :
. par agitation ou
. par une étape de dispersion qui est réalisée au moyen d'un rotor de type Cowles ou d'un rotor à lames, de préférence un rotor à lame de scie, qui peut percuter les particules solides de chitosane et/ou de dérivés de celui-ci à grande vitesse, et
- pour faciliter la réticulation UV du chitosane et/ou du dérivé, ladite composition d'encollage est enrichie avec des agents de réticulation à monomères double liaison supplémentaires comprenant des monomères acryliques à faible impact environnemental ajoutés dans une quantité égale au pourcentage m/v de chitosane et/ou de dérivés de celui-ci dans la composition d'encollage.

2. Composition d'encollage selon la revendication 1, ladite composition d'encollage étant, pour faciliter la réticulation UV du chitosane et/ou du dérivé, enrichie avec des agents de réticulation supplémentaires comprenant :
. des huiles siccatives, de préférence de l'huile de lin constituée d'acide oléique et linoléique, et/ou
. des acides polycarboxyliques.

3. Composition d'encollage selon la revendication 1 ou 2, dans laquelle ladite solution d'acide organique avec un pH inférieur à 6,5 à 3-9 % v/v, est une solution d'acide acétique, d'acide citrique, d'acide pyruvique ou d'acide tartrique.

4. Composition d'encollage selon la revendication 1, 2 ou 3, dans laquelle le degré de désacétylation dudit chitosane et/ou desdits dérivés de celui-ci est de 75 à 85 %.

5. Composition d'encollage selon la revendication 1, 2, 3 ou 4, dans laquelle le chitosane et/ou les dérivés de celui-ci sont dans un état solide, de préférence de la poudre, des granulés ou des paillettes, ou dans un état fluide, par exemple sous la forme d'une pâte à haute densité, avant d'être dissous par agitation et/ou dispersion dans ladite solution contenant un acide organique avec un pH inférieur à 6,5 à 3 à 9 % v/v.

6. Composition d'encollage selon l'une quelconque des revendications 1 à 5, dans laquelle ladite solution de chitosane et/ou de dérivés de celui-ci dans un acide organique, avec un pH inférieur à 6,5, comprend de la colle d'amidon et/ou de poisson dans une proportion de 1:1 par rapport à la quantité de chitosane et/ou de dérivés de celui-ci.

7. Composition d'encollage selon l'une quelconque des revendications 1 à 6, dans laquelle :
- ladite composition d'encollage comprend :
- des huiles siccatives, de préférence de l'huile de lin constituée d'acide oléique et linoléique, et/ou
- des acides polycarboxyliques, de préférence comprenant de l'acide citrique ajouté dans une quantité d'au plus 2 % basée sur la quantité de chitosane sec dans la composition d'encollage.

8. **Procédé de préparation d'une composition d'encollage** pour des fibres et fils et/ou des étoffes fabriquées à partir de telles fibres, en particulier pour des fibres naturelles animales, des fibres végétales, des fibres polymères synthétiques, des fibres polymères naturelles de fabrication humaine, des filaments continus d'origine animale et/ou des filaments discontinus d'origine animale, destinés à être utilisés dans un état pur ou mélangés les uns avec les autres, dans lequel ladite composition d'encollage comprend :
- du chitosane et/ou des dérivés de celui-ci présentant une masse moléculaire Mᵥ allant de 120.000 Da à 180.000 Da, de préférence une masse moléculaire Mᵥ de l'ordre de 150.000 Da, avec un degré de désacétylation de 70 à 90 %, et une viscosité à température ambiante de 20 à 200 cps avec 1 % m/m de chitosane dans 1 % m/v d'acide acétique ou citrique et
- une solution d'acide organique avec un pH inférieur à 6,5 à 3-9 % v/v, dans laquelle sont dissous 3 % à 9 % m/v dudit chitosane et/ou desdits dérivés de celui-ci, ladite composition d'encollage étant soumise à une étape de dissolution par dispersion réalisée à l'aide de moyens de dispersion qui sont aptes à obtenir une dispersion fine du chitosane et/ou des dérivés de celui-ci présents dans la composition d'encollage par des impacts à haute vitesse avec les particules solides de chitosane et/ou de dérivés de celui-ci présents dans le bain, jusqu'à dissolution desdites particules solides de chitosane et/ou de dérivés de celui-ci dans le bain, lesdits moyens de dispersion pour réaliser ladite étape de dispersion du chitosane et/ou des dérivés de celui-ci comprenant au moins un rotor de type Cowles ou un rotor à disque denté comportant des lames, les dents étant formées par des lames, de préférence présentant la forme de dents de scie,
dans lequel, pour faciliter la réticulation UV du chitosane et/ou du dérivé, ladite composition d'encollage est enrichie avec des agents de réticulation à monomères double liaison supplémentaires comprenant des monomères acryliques ajoutés dans une quantité égale au pourcentage de chitosane et/ou de dérivés de celui-ci dans la composition d'encollage.

9. Procédé de préparation d'une composition d'encollage selon la revendication 8, dans lequel ladite étape de dispersion de chitosane et/ou de dérivés de celui-ci est réalisée en introduisant le bain dans lequel ont été ajoutés le chitosane et/ou les dérivés de celui-ci dans un état solide ou fluide, dans une cuve d'un disperseur dans lequel ledit rotor Cowles ou ledit rotor à lames est à rotation, de préférence à une vitesse périphérique de rotation du rotor supérieure à 10 mètres/seconde et inférieure à 40 m/seconde, de préférence à une vitesse périphérique du rotor de 13 à 32 mètres/seconde.

10. Procédé de préparation d'une composition d'encollage selon l'une quelconque des revendications 8 à 9, dans lequel ledit chitosane et/ou lesdits dérivés de celui-ci sont dissous par agitation ou par dispersion dans ladite composition d'encollage à partir d'un état solide, de préférence de la poudre, des granulés ou des paillettes, ou d'un état fluide, de préférence sous la forme d'une pâte à haute densité.

11. Procédé de préparation d'une composition d'encollage selon l'une quelconque des revendications 8 à 10, dans lequel ladite solution de chitosane et/ou de dérivés de celui-ci dans un acide organique, avec un pH inférieur à 6,5, comprend de la colle d'amidon et/ou de poisson dans une proportion de 1:1 par rapport à la quantité de chitosane et/ou de dérivés de celui-ci.

12. Procédé de préparation d'une composition d'encollage selon l'une quelconque des revendications 8 à 11, dans lequel, pour faciliter la réticulation UV du chitosane et/ou du dérivé, ladite composition d'encollage est enrichie avec des agents de réticulation supplémentaires comprenant :
- des huiles siccatives, de préférence de l'huile de lin constituée d'acide oléique et linoléique, et/ou
- des acides polycarboxyliques.

13. Procédé de préparation d'une composition d'encollage selon la revendication 8 ou 12, dans lequel lesdits acides polycarboxyliques comprennent de l'acide citrique ajouté dans une quantité d'au plus 2 % basée sur la quantité de chitosane sec dans la composition d'encollage.

14. **Procédé de réticulation de chitosane et/ou de dérivés de celui-ci** présents dans la composition d'encollage selon l'une quelconque des revendications 1 à 7, sur des fibres imprégnées avec ladite composition d'encollage, dans lequel ladite étape de réticulation est réalisée :
- en exposant les fibres imprégnées avec ladite composition d'encollage au rayonnement d'une lampe UV et
- par traitement chimique.

15. Procédé de réticulation de chitosane et/ou de dérivés de celui-ci selon la revendication 14, dans lequel ladite étape de réticulation est réalisée en exposant lesdites fibres imprégnées avec ladite composition d'encollage au rayonnement d'une lampe UV :
- ayant une puissance de 400 W à 600 W, de préférence une puissance d'environ 500 W, et
- ayant une intensité de 10 mV/cm² à 30 mV/cm², de préférence une intensité d'environ 20 mV/cm²,
pendant un temps d'exposition allant de 20 à 80 secondes, de préférence pendant un temps d'exposition allant de 30 à 65 secondes, à une distance de la lampe UV allant de 15 cm à 30 cm, de préférence à une distance de la lampe UV de l'ordre de 20 cm.
